



US007681305B2

(12) **United States Patent**  
**Hopper**

(10) **Patent No.:** **US 7,681,305 B2**  
(b5) **Date of Patent:** **Mar. 23, 2010**

(54) **METHOD OF MAKING IGNITION WIRE  
WITH GRAFTED COATING**

4,000,362 A 12/1976 Kawaguchi et al.  
4,008,113 A 2/1977 Glander et al.  
4,435,692 A 3/1984 Miyamoto et al.  
4,471,215 A 9/1984 Blumer  
4,700,171 A 10/1987 Coffey et al.

(75) Inventor: **Bradley T. Hopper**, Monticello, AR  
(US)

(73) Assignee: **Federal-Mogul World Wide, Inc.**,  
Southfield, MI (US)

(\*) Notice: Subject to any disclaimer, the term of this  
patent is extended or adjusted under 35  
U.S.C. 154(b) by 0 days.

(21) Appl. No.: **11/591,256**

(22) Filed: **Nov. 1, 2006**

(65) **Prior Publication Data**

US 2007/0044302 A1 Mar. 1, 2007

**Related U.S. Application Data**

(62) Division of application No. 11/175,058, filed on Jul. 5, 2005, now Pat. No. 7,148,422.

(60) Provisional application No. 60/585,125, filed on Jul. 2, 2004.

(51) **Int. Cl.**

*H01B 13/00* (2006.01)

*H01B 13/06* (2006.01)

*H01B 13/32* (2006.01)

(52) **U.S. Cl.** ..... **29/825**; 29/828; 174/120 R;  
427/118

(58) **Field of Classification Search** ..... 29/825,  
29/828; 174/120 R, 120 C, 120 SR, 122 R;  
338/214; 427/118

See application file for complete search history.

(56) **References Cited**

**U.S. PATENT DOCUMENTS**

1,830,411 A 11/1931 Schork, Jr.  
2,992,292 A \* 7/1961 Brown ..... 174/112  
3,258,522 A 6/1966 Bartos et al.  
3,484,540 A 12/1969 Wilson et al.

(Continued)

**FOREIGN PATENT DOCUMENTS**

GB 777552 6/1957

(Continued)

*Primary Examiner*—A. Dexter Tugbang

*Assistant Examiner*—Livius R Cazan

(74) *Attorney, Agent, or Firm*—Robert L. Stearns; Dickinson Wright, PLLC

(57) **ABSTRACT**

An ignition wire includes a conductive core, an insulation layer surrounding the core, an insulating jacket surrounding the insulation layer and a coating layer which is grafted and bonded to at least a portion of an exterior surface of the insulating jacket. The coating layer and insulating jacket are preferably formed of silicone materials. The coating layer is operative to provide enhanced resistance to heat and abrasion, as well as other benefits to the exterior surface of the insulating jacket. The coating layer may be transparent and provide an aesthetically pleasing clear coat, or may be tinted or colored to produce various other cosmetic or decorative characteristics to the outer surface of the ignition wire. The coating layer provides these enhanced protections without the diminishing electrical or mechanical performance properties of either the insulation layer or the insulating jacket. The coating layer is also adapted to provide protection to a cosmetic layer which may be applied to the exterior surface of the insulating jacket.

**10 Claims, 1 Drawing Sheet**



**US 7,681,305 B2**

Page 2

---

U.S. PATENT DOCUMENTS

|               |         |                           |
|---------------|---------|---------------------------|
| 4,704,596 A   | 11/1987 | Coffey et al.             |
| 4,732,722 A   | 3/1988  | Aida et al.               |
| 4,769,287 A   | 9/1988  | Zaopo et al.              |
| 4,801,766 A   | 1/1989  | Aida et al.               |
| 4,814,546 A   | 3/1989  | Whitney et al.            |
| 5,057,812 A * | 10/1991 | Yukawa et al. .... 338/66 |
| 5,059,938 A   | 10/1991 | Brown                     |
| 5,217,553 A   | 6/1993  | Marx et al.               |

|                 |         |                             |
|-----------------|---------|-----------------------------|
| 5,977,489 A     | 11/1999 | Crotzer et al.              |
| 6,521,695 B1    | 2/2003  | Peruzzotti et al.           |
| 6,630,244 B1 *  | 10/2003 | Mao et al. .... 428/447     |
| 6,783,865 B2 *  | 8/2004  | Sanduja et al. .... 428/523 |
| 2006/0004170 A1 | 1/2006  | Sanduja et al.              |

FOREIGN PATENT DOCUMENTS

|    |         |        |
|----|---------|--------|
| JP | 7-37434 | 2/1995 |
|----|---------|--------|

\* cited by examiner



FIG. - 1



FIG. - 2

## METHOD OF MAKING IGNITION WIRE WITH GRAFTED COATING

### CROSS-REFERENCES TO RELATED APPLICATIONS

This patent application claims priority to U.S. Provisional Patent Application Ser. No. 60/585,125, filed Jul. 2, 2004 and U.S. patent application Ser. No. 11/175,058, now U.S. Pat. 7,148,422, both of which are hereby incorporated herein by reference in their entirety.

### BACKGROUND OF THE INVENTION

#### 1. Field of the Invention

The present invention relates generally to insulated electrical conductors and, in particular, to a method for making abrasion resistant ignition wires for spark plugs and similar ignition devices.

#### 2. Related Art

Ignition wires for spark plugs commonly include a conductive core, a conductor or semi-conductor coating layer, a release coating, an electrical insulation layer, a strengthening layer to provide enhanced tensile strength and an insulating outer sheath or jacket, and may also include various adhesive and other inner layers. The outer jacket also frequently includes a cosmetic or decorative layer or printed portion on its outer surface. The layers described above may be arranged in different combinations and orders and their particular arrangement will vary depending on the intended application environment and other factors.

In addition to various solid or stranded metal wire configurations, the conductive core may also comprise a wire-wound configuration. Wire-wound cores typically have a braided or otherwise woven insulating core member, such as a rope, to provide tensile strength. This member may have a ferrite or other coating applied that is in turn wrapped with a metal wire and coated with an adhesive and/or conductive or semi-conductive layer. Examples of such wire wound conductive cores are taught by Miyamoto et al. in U.S. Pat. No. 4,435,692 and Coffe et al. in U.S. Pat. No. 4,700,171. Miyamoto et al. teach a wire wound ignition cable in which a resistance wire is wound over a woven member, such as a woven aramid string, which has been coated with a chlorinated polyethylene/ferrite mixture to provide the conductive core. The resistance wire and ferrite coated core are in turn coated by a woven strengthening member and an extruded sheath of a blend of polyethylene and ethylene propylene diene monomer (EPDM). Coffe et al. discloses an ignition cable similar in some respects to that taught by Miyamoto et al. in which a conductive core is formed by dip coating a strengthening member formed from a glass fiber bundle with an insulating layer containing a mixture of EPDM and magnetic particles, such as iron oxide. The coated woven core is then helically wrapped with a resistance wire conductor, such as various Ni alloys. The resistance wire of Coffe et al. is then dip coated with a semi-conductive thermoplastic polymer, such as a silicone or acrylic polymer. The semi-conductive thermoplastic polymer contains carbon particles and release agents which allow subsequently applied insulating layers to be stripped away cleanly. The conductive core of Coffe et al. is coated with an insulating layer formed from EDPM, an optional fiberglass braid layer, and a polymer jacket formed from a mixture of EPDM, ethylene vinyl acetate copolymer, phenolic antioxidant and a metal salt antioxidant. In general, for conductive cores as described in Miyamoto et al. and Coffe et al., a release coating is applied to the exterior of the core or incor-

porated into a conductive coating in order to promote removal of the insulating layer from the core during the application of terminations or connectors to the ignition wire.

The ignition wire insulation layer may be made from various materials that provide electrical insulation and are resistant to degradation at the elevated operating temperatures of an internal combustion engine. Examples of materials that have been used for the insulating layer in various wire configurations include EPDM and various silicones.

10 The strengthening layer is typically made from fiberglass and comprises a woven sheath. This layer may be woven over the insulation layer directly or pre-woven and applied over the insulation layer.

15 The insulating jacket is typically made of a material that is resistant to high levels of heat, as well as abrasion, because it forms the outer wall of the ignition wire. Various materials have been used for the insulating jacket, such as EPDM, various silicones and other materials, depending on the intended application and other factors. The jacket is typically

20 extruded over the insulation layer. The process of extrusion can alter the thermal, mechanical and/or chemical properties of both the jacket and the underlying insulation layer. As such, the overall appearance of the outer surface of the jacket may be affected, as well as the abrasion resistance of the jacket itself.

25 As noted above, in many ignition wire applications, it is desirable to apply cosmetic or decorative materials, such as various inks and the like, which are used to print information on the wire such as the manufacturer's name, product numbers, wire sizes, manufacturer's logos or trademarks, performance characteristics, specifications, or other important information, as well as ornamental designs. Being located on the outer surface, such materials are subject to high temperatures, abrasion from dirt and other under-hood sources of abrasion, mechanical stress, chemicals and other agents which promote their degradation.

30 To improve the mechanical, thermal and chemical properties of the insulated wires, the jacket may include a coating material coated thereon. U.S. Pat. No. 4,000,362 to Kawaguchi et al. discloses an electrical insulated metallic wire comprising a releasing layer coated on the metallic wire with a baked-on insulating layer superposed on the releasing layer. The insulating layer is formed on the releasing layer by coating and baking a silicone-containing insulating varnish having a releasing ability on the releasing layer. The releasing ability of the silicone-containing insulating varnish allows the insulating layer to be easily stripped from the releasing layer. It is believed that the construction of Kawaguchi would not be applicable for the protection of the cosmetic or decorative materials or enhancing the abrasion resistance of the jacket because it is applied over a release coating and is designed to be readily removed from the outer surface of the wire jacket.

35 Therefore, it is desirable to develop ignition wires with improved protection, such as improved heat and abrasion resistance, to the outer surface of the jacket. Further, it is also desirable to develop ignition wires with enhanced protection for cosmetic or decorative materials, such as inks, that are applied to the outer surface of the wire jacket.

### SUMMARY OF THE INVENTION

65 In one aspect, the present invention is an ignition wire having a coating layer which is chemically grafted and bonded to the exterior surface of an insulating jacket. Still further, the coating layer may be transparent and afford advantages for use in providing a clear coat on the outer surface of the insulating jacket layer as well as use in con-

junction with a cosmetic layer applied to this surface. The coating layer is adapted to provide improved resistance to abrasion to the insulating jacket. The coating also provides an aesthetically pleasing surface finish, such as a clear-coat finish on the exterior surface of the ignition wire.

In a second aspect, the present invention comprises an ignition wire which includes a conductive core, an insulation layer composed of an insulating substrate surrounding the conductive core, an insulating jacket surrounding the insulation layer, and a coating layer chemically grafted and bonded to at least a portion of an outer surface of the insulating jacket. The insulating jacket may also include a cosmetic layer applied to its outer surface such that the coating layer also provides similar protection to the cosmetic layer as it does to the insulating jacket.

In a third aspect, the coating layer, insulating jacket and insulation layer are preferably formed from silicones.

In a fourth aspect, the coating layer provides enhanced resistance to abrasion of the insulating jacket without deteriorating the electrical or mechanical performance characteristics of either the insulation layer or the insulating jacket.

#### BRIEF DESCRIPTION OF THE DRAWINGS

These and other features and advantages of the present invention will become more readily appreciated when considered in connection with the following detailed description and appended drawings, wherein:

FIG. 1 is a prospective view of an ignition wire of the present invention; and

FIG. 2 is a cross-sectional view taken along line 2-2 of the ignition wire of FIG. 1.

#### DETAILED DESCRIPTION OF THE PREFERRED EMBODIMENT

In reference to FIGS. 1-2, an ignition wire 10 comprises a conductive core 12 surrounded by an insulation layer 14 and a jacket 18 having an outer surface 20, which includes a cosmetic layer 22, and a silicone-containing coating layer 24 that is grafted, using chemical or physical grafting processes, and bonded thereon to thereby improve the abrasion and heat resistance of the ignition wire 10 without adversely affecting the mechanical, thermal and/or chemical properties of the underlying insulation layer 14, jacket 18 or cosmetic layer. The insulation layer 14 is an insulating material that is extruded over the conductive core 12. A strengthening member, such as fiberglass braid 16, is then applied over the insulation layer 14 for mechanical strength. The jacket 18 is extruded over the braided layer 16 and is composed of an insulating material that improves the resistance of the ignition wire 10 to extreme levels of heat as well as providing additional electrical insulation. The silicone-containing coating material is grafted and bonded to the jacket 18.

The conductive core 12 can be provided as an electrically conductive metal wire or wire strand, a flexible, single, carbon fiber or strand of fibers, a wire-wound bundle of braided or woven fibers having a ferrite or other coating, or any other electrically conductive wire configuration of a type commonly used for ignition wires and/or cables. Preferably, the core 12 is a wire-wound Kevlar core having a ferrite coating with a Cu—Ni alloy (12% Ni/88% Cu by weight) wire wound around it. The Kevlar core may comprise a braided rope or string configuration such as, for example, a Kevlar string having a diameter of about 0.035 inches (Kevlar DT140) with a ferrite coating on its outer surface. A preferred ferrite coating comprises a mixture of Cu—Zn ferrite particles having

average particle size of about 200-300 mesh and comprising about 40% by weight in a polymer matrix. While Cu—Zn ferrite was utilized, other ferrites are also believed to be suitable for use, as they all will tend to produce a magnetic field in response to current flow in the wire windings, thereby increasing the inductance and electromagnetic interference suppression of the wire. The polymer matrix may include both conductive and non-conductive polymers that are suitable for use in the ignition wire application environment, including those made from conductive and non-conductive latex materials. An example of a suitable conductive latex is WC 2193 manufactured by Key Polymer. In a preferred configuration, the Cu—Ni alloy wire has a wire diameter of about 0.0035 inches (39gauge) and is wrapped around the ferrite-coated Kevlar core with a winding density of about 147 windings/inch. The wire wound conductive core 12 may then be coated with a commercially available conductive latex material and a release agent of types well-known in the art, such as conductive latex materials EFTEC WB 2693 manufactured by HB Fuller or WC 2193 manufactured by Key Polymer, and release agent Grafo 1145 (manufactured by Fuchs Lubricants Co.). The diameter of the conductive core 12 is about 0.058 inch (+/-10%) having a resistance of about 170ohms/ft (+/-10%).

The insulation layer 14 is extruded over the core 12 and provides an insulating layer to electrically isolate and mechanically protect the core 12. The mechanical bond formed by the extrusion process is relatively weak so that the insulation layer 14 can be easily stripped from the conductive core 12. The insulation layer 14 has a thickness of about 0.061 inches (+/-0.005 inches) and is composed of a flexible insulating thermoset polymer material of a type used in ignition wires and/or cables, such as various insulating elastomers, including various silicones, EPDM and other insulating elastomers having suitable mechanical strength, heat resistance, electrical isolation and other characteristics required in ignition applications. Preferably, the insulation layer 14 is composed of silicone or a silicone-containing elastomer substrate. The methods and equipment used to extrude the materials used for insulation layer 14 are well-known. In an exemplary embodiment, insulation layer 14 comprised GS67FM silicone manufactured by Specialty Products and Polymers, Inc.

The fiberglass braiding layer 16 is responsible for providing the ignition wire 10 with mechanical strength. In an exemplary embodiment, the fiberglass braid layer 16 was composed of a natural glass fiber yarn having a standard basket weave of 8.5 ppi. The fiberglass braid 16 may be braided directly over the surface of the insulation layer 14, but may also be applied by inserting the wire containing the insulation layer into a pre-woven sheath. The braided pattern can be a woven pattern, a simple helical pattern, or the like, such as is commonly used in ignition wires and/or cables.

The insulating jacket layer 18, which is extruded over the fiberglass braiding layer 16, is responsible for providing further electrical insulation or isolation and resistance to heat and abrasion of the exterior surface of the ignition wire 10. The jacket 18 is composed of a flexible insulating thermoset polymer material of a type used in ignition wires and/or cables, such as various insulating elastomers, including various silicones and other insulating elastomers having suitable mechanical strength, heat resistance, electrical isolation and other characteristics required in ignition applications. Preferably, insulating jacket layers 18 is made of a silicone compound that functions over the entire temperature range commonly used to test vehicles and their ignition wires and can, for example, withstand elevated temperatures in the range of 425° F. to 600° F. or more, while also retaining flexibility and

desirable electrical performance characteristics at temperatures well below  $-58^{\circ}$  F. The insulating jacket layer **18** is preferably slightly thicker than insulation layer **14** and in one embodiment had a thickness of about 0.077 inches ( $+/-0.005$  inches). In an exemplary embodiment, insulating jacket **18** was made by extruding GS810LC silicone manufactured by Specialty Products and Polymers, Inc. Insulating jacket layer **18** may also incorporate a dye or other colorant which may be used to control the color of jacket **18**, and in particular, the color of the exterior surface **20** of jacket **18**. Table 1 illustrates the dimensions of a number of ignition wires of the present invention having the general construction described above, including a silicone insulation layer and silicone insulating jacket layer.

outer surface of the insulating jacket layer. However, it is believed that coating layer **24** may also incorporate various known tints, colorants and the like that may be used to make the layer translucent or even opaque in character, and to provide a wide variety of tints, shades and colors. Coating layer **24** may be formed using any coating material composition that is operative to produce a grafted and bonded coating layer to insulating jacket layer **18**. Grafting preferably utilizes chemical grafting processes, but various physical grafting processes have also been suggested for other applications and may be extendable for use in the present invention. When insulating jacket layer **18** comprises a silicone, coating layer **24** also preferably comprises a grafted and bonded silicone.

TABLE 1

| Wire Diameter (mm) | Conductor Type    | Core Diameter (inches) | Insulation Layer        |               | Insulating Jacket Layer |               |
|--------------------|-------------------|------------------------|-------------------------|---------------|-------------------------|---------------|
|                    |                   |                        | Outer Diameter (inches) | Wall (inches) | Outer Diameter (inches) | Wall (inches) |
| 5                  | wire wound        | 0.058                  | 0.120                   | 0.031         | 0.201                   | 0.041         |
| 7                  | wire wound        | 0.058                  | 0.0180                  | 0.061         | 0.276                   | 0.048         |
| 7                  | metallic          | 0.056                  | 0.180                   | 0.062         | 0.276                   | 0.048         |
| 7                  | conductive        | 0.070                  | 0.180                   | 0.055         | 0.276                   | 0.048         |
|                    | carbon/fiberglass |                        |                         |               |                         |               |
| 8                  | wire wound        | 0.058                  | 0.205                   | 0.074         | 0.315                   | 0.055         |
| 8                  | conductive        | 0.070                  | 0.205                   | 0.068         | 0.315                   | 0.055         |
|                    | carbon/fiberglass |                        |                         |               |                         |               |

The ignition wire construction of the present invention is believed to be extendable and applicable to any ignition wire size.

The surface **20** of the jacket **18** can be surface finished in a variety of colors using a variety of different materials, finishes and techniques, such as the printing of various inks, the use of shrink-wrap appliqués, embossing and the like, to achieve a desired and enhanced exterior cosmetic or decorative layer **22** appearance for the ignition wire **10**. The color or other physical characteristics of cosmetic layer **22** may be selected to provide contrast to or otherwise enhance the appearance of the outer surface **20** of insulating jacket **18**. Cosmetic or decorative layer **22** can take many forms, including printed information such as the manufacturer's name, product numbers, wire sizes, manufacturer's logos or trademarks, performance characteristics, specifications or other important information, as well as a broad array of ornamental designs. For example, the silicone-containing jacket **18** may include a colorant to produce a dark blue color, while cosmetic layer **22** can be printed with a silver ink to provide contrasting silver-colored lettering on the jacket surface **20**.

To provide the ignition wire **10** with improved resistance to abrasion and heat and to help maintain and/or enhance the aesthetic or cosmetic appearance of the jacket surface **20** and any cosmetic or decorative layer **22** that is applied, a coating layer **24** is applied over the jacket surface **20**. The coating layer **24** is preferably a relatively thin (i.e., microns thick) layer of a transparent, silicone-based or silicone-containing coating material. In a preferred embodiment, coating layer **24** is between about 5-40 microns thick. Coating layer **24** is grafted and bonded, such as by using chemical grafting processes, to the outer surface **20** of insulating jacket layer **18** with strong covalent chemical bonds. Coating layer **24** is preferably a transparent coating, and even more preferably a clear coating, such that it provides a clear coat finish to the

A preferred coating layer **24** may be formed from the coating material composition described in more detail in Example 1 below.

## EXAMPLE 1

A preferred transparent coating layer **24** may be made from a coating material composition which includes between 35 and 45 parts by weight of a silicone prepolymer, less than 1 part by weight of a silane coupling agent, less than 1 part by weight of a catalyst, less than 1 part by weight of a graft initiator and the balance a reactive solvent.

The silicone prepolymer is preferably an RTV silicone that is adapted upon curing to provide a silicone polymer coating layer **24**. The coupling agent is preferably a silane coupling agent, and more preferably an amino-functional silane coupling agent. The catalyst is preferably operative to promote grafting by polymerization of the silicone polymer coating **24** to the outer surface of insulating jacket layer **18**. The graft initiator is operative to prepare the outer surface of the insulating jacket layer to receive by grafting a coating layer comprising the silicone prepolymer and said coupling agent. It is believed that the graft initiator is adapted to produce graft receptor sites on the insulating jacket layer by alteration of the chemical bonds of the silicone material of insulating jacket layer **18** at its outer surface **20**.

A preferred coating material composition includes: 40.00 parts by weight of silicone prepolymer, preferably DC 1-2620 (manufactured by Dow Corning) which is a one part RTV methoxy siloxane silicone resin solution comprising, by weight, >60% octamethyltrisiloxane, 15.0-40.0% dimethyl methylphenylmethoxy siloxane, 3.0-7.0% methyltrimethoxysilane and 3.0-7.0% toluene and is described as being operative to produce elastoplastic conformal coatings;

60.00 parts by weight of a reactive solvent DC OS-30 (manufactured by Dow Corning) which is a methyl siloxane liquid comprising, by weight >60% decamethyltetrasiloxane;

0.25 parts by weight of monomer silane Silquest A-1100 (manufactured by GE Silicones) which is gamma aminopropyltriethoxysilane as a coupling agent;

0.10 parts by weight of methyl ethyl ketone (MEK) peroxide (0.01% in MEK) organic catalyst in plasticizers comprising, by weight, about 58.0% 2,2,4 trimethyl-1,3-pentanediol diisobutyrate, 32-34% methyl ethyl ketone peroxide, 6.0% hexylene glycol, 1-2% methyl ethyl ketone, 0.7% hydrogen peroxide and 0.7% water; and

0.10 parts by weight of silver perchlorate (0.01% in toluene).

This is further shown in Table 2 below, as well as by weight percent of the various constituents:

TABLE 2

| Coating Material Composition Constituent | Parts     | Percent   |
|------------------------------------------|-----------|-----------|
| Dow Corning OS-30                        | 60.00000  | 59.73121  |
| Dow Corning 1-2620                       | 40.00000  | 39.82081  |
| Lupersol DDM-9 MEKP                      | 0.00001   | 0.00001   |
| Methyl Ethyl Ketone                      | 0.09999   | 0.09954   |
| Silquest A-1100                          | 0.25000   | 0.24888   |
| Silver Perchlorate                       | 0.00001   | 0.00001   |
| Toluene                                  | 0.09999   | 0.09954   |
| Total                                    | 100.45000 | 100.00000 |

The coating material composition used for coating layer 24 is prepared by stirring each component, in the preferred concentration ratio (in parts by weight) using the method described below.

First, the method included a step of forming a graft precursor polymer. To form a graft precursor polymer, silane coupling agent is stirred into a portion of the silicone prepolymer. These constituents were thoroughly blended together by stirring using a mixer to achieve a homogenous batch. After blending, mixture was allowed to stand for a period of time sufficient for the silane coupling agent to form chemical bonds with or graft to the silicone prepolymer, thereby forming a graft precursor polymer. In this case where the silicone prepolymer was a one part RTV methoxy siloxane silicone resin solution of DC 1-2620, and the coupling agent was a monomer silane of gamma aminopropyltriethoxysilane in the form of Silquest A-1100, a sufficient time was about 24 hours. It is believed that the silane monomer grafts to the silicone prepolymer and forms a comb-like molecular structure on the polymer which also functions as graft initiator sites for a subsequent grafting reaction of the graft precursor polymer to the outer surface of the insulating jacket layer. By use of a portion of the silicone prepolymer, it is meant that use of roughly an equal portion (by volume or by weight) of the prepolymer and the coupling agent are mixed to form the graft precursor polymer is preferred. While these quantities are preferred, either a lesser quantity of prepolymer, or a greater quantity of prepolymer may be used to make graft precursor polymer.

Secondly, following the step of forming the graft precursor polymer, the method included a step of mixing the balance of the silicone prepolymer and the reactive solvent for a time sufficient to thoroughly mix them. In one embodiment, the

mixing time was about 5 minutes. This will of course vary as a function of the mixing speed and the like.

Thirdly, following the mixing together of the silicone prepolymer, silane monomer and reactive solvent, the graft polymerization catalyst in the form of MEK peroxide was added and again thoroughly mixed together with these components by stirring in a mixer for between about 10 minutes.

Fourthly, the graft precursor polymer, which had been allowed to set for a sufficient time as described above was 10 added and mixed together into the batch for about 15 minutes.

Fifthly, the graft initiator in the form of silver perchlorate in toluene was added and again thoroughly mixed together with the other components by stirring in a mixer for about 30 minutes.

15 The coating material composition was then applied by dip coating then and chemically bonded to the insulating jacket layer 12 by chemical grafting or graft polymerization. While dip coating was employed, spray coating and other known coating methods may be used. By chemical grafting, it is 20 meant that some degree of cross-linking and covalent bonding occurs between the coating material composition of coating layer 24 and the outer surface 20 of insulating jacket layer 18.

Specifically, insulating jacket layer 18 of wire 10 was 25 dipped into a supply of the coating material composition and then partially cured in an oven operated at a temperature of between 650-800° F. or about 0.5 minutes or less. The ignition wire 10 was then sent through a water bath to cool back down to room temperature. Since the completion of the graft and/or 30 curing of the silicone prepolymer process takes about 72 hours to complete a silicone-based lubricant may be applied to the coated layer 16 surface to prevent the ignition wire from sticking to other surfaces until the curing/grafting is complete. In this way, ignition wire 10 can be further handled or 35 otherwise used before the silicone polymer coating layer 24 is completely cured.

Unlike mechanical bonds formed between core 12 and insulation layer 14, as well as between insulation layer 14 or, when utilized, strengthening layer 16 and insulating jacket layer 18, the strong chemical bonds formed between the insulating jacket layer 18 and coating layer 24 by grafting greatly contributes to improved resistance of the insulating jacket layer 18 to abrasion, as well as improved heat resistance of the ignition wire 10, thereby significantly improving 40 the usable life of the ignition wire. Since the cured coating material composition of coating layer 24 is preferably transparent, the outer surface 20 of insulating jacket layer 18 can be cosmetically enhanced prior to grafting by the addition of cosmetic layer 22, and, unlike the use of extrusion processes 45 to add a protective layer such as coating layer 18, the grafting process of the present invention does not change the cosmetic appearance of the outer surface 20 of insulating jacket layer 18, or cause the removal or distortion of, or otherwise undesirably affect, cosmetic layer 22. These advantages are 50 obtained using the insulating jacket layer 18 and the specific cured coating material composition of coating layer 24 of the present invention without adversely affecting the mechanical, thermal and/or chemical properties of the insulating jacket layer 18, the underlying insulation layer 14, or cosmetic layer 22. Coating layer 24 also provides an aesthetically desirable 55 finish to the exterior of ignition wire 10. This aesthetically pleasing appearance is analogous in this regard to the application of a clear-coat layer applied to the exterior of painted or otherwise colored surfaces, such as are widely used to enhance the exterior appearance of automobiles, various watercraft, recreational vehicles and other items. Coating layer 24 may be applied to all of the exterior surface 20 of

ignition wire 10, or only a portion or portions thereof. Preferably, coating layer 24 will be applied to the entire outer surface 20 of ignition wire 10 so as to maximize the protections afforded to this surface, as described herein. It is preferred that coating layer 24 is transparent, such that an underlying cosmetic or decorative layer 22 is visible through coating layer 24. It is further preferred that in addition to being transparent, coating layer is substantially clear or uncolored to provide a clear-coat over outer surface 20 of insulating jacket layer 18. However, it will be understood that coating layer 24 may also incorporate all manner of colorants, tints and the like so as to color or shade this layer, and the same may be included in varying concentrations and colors such that this layer may be translucent or still further substantially or completely opaque. Such is the range of appearances that may be achieved in chemically grafted and bonded coating layer 24.

An external cosmetic or decorative layer like unto that described above for cosmetic layer 22 may also be applied to the outer surface of transparent coating layer 24. While some of the protection benefits described are believed to be reduced in such a configuration as compared to that of cosmetic layer 22, some applications may require or make highly desirable the application of a cosmetic layer to the exterior surface of wire 10 and coating layer 24. It will also be appreciated that cosmetic layer 22 and external cosmetic layer may each be implemented separately or that they may be implemented together and in various combinations.

It will thus be apparent that there has been provided in accordance with the present invention an ignition wire for spark plugs and similar ignition devices and a method for manufacturing the same that achieves the aims and advantages specified herein. Further, the present invention also describes a coating material composition for application to ignition wires for spark plugs and similar ignition devices and a method of making the same. It will, of course, be understood that the foregoing description is of a preferred exemplary embodiment of the invention and that the invention is not limited to the specific embodiment shown and/or described. For example, the grafting technique may include irradiation or compressive bonding processes to fully cure and graft the coating layer 20 to the jacket 18. It has also been suggested that these and other techniques, such as those described in U.S. Pat. No. 6,630,644, which is hereby incorporated herein by reference in its entirety, may be employed to promote grafting and bonding of a coating layer largely by utilization of physical processes as compared to chemical grafting processes. Such grafting techniques may also be utilized in conjunction with the present invention. Still further, the present invention is also believed to be extendable to insulating jacket materials other than silicone jacket materials, such as those made from EPDM or various chlorinated polyethylene elas-

tomers (CPE), as well as co-polymers of these materials and various silicones, depending on the application requirements for ignition wire 10.

Obviously, many modifications and variations of the present invention are possible in light of the above teachings. It is, therefore, to be understood that within the scope of the appended claims, the invention may be practiced otherwise than as specifically described.

What is claimed is:

- 10 1. A method of making an ignition wire (10), comprising the steps of:
  - forming a conductive core (12);
  - forming an insulation layer (14) so as to surround the conductive core (12);
  - providing a strengthening member (16) of braided fibers so as to surround the insulation layer (14);
  - forming an insulating jacket (18) so as to surround the strengthening member (16), the insulating jacket (18) having an outer surface (20);
  - 20 forming a coating layer (24) so as to surround at least a portion of the outer surface (20) of the insulating jacket (18);
  - and grafting and chemically bonding the coating layer (24) to the outer surface (20) of the insulating jacket (18) so that covalent bonds develop between their respective atoms.
- 20 2. The method of claim 1, wherein said step of forming the coating layer comprises applying the coating layer to the outer surface of the insulating jacket using a pre-polymer solution by at least one of dip-coating or spray coating.
- 25 3. The method of claim 2, wherein the pre-polymer solution comprises a silicone pre-polymer solution.
- 30 4. The method of claim 3, wherein the silicone pre-polymer solution comprises a solution of a silicone pre-polymer, a reactive solvent, a silane monomer, and a catalyst, wherein the catalyst is operative to catalyze polymerization and the grafting of said coating layer to said insulating jacket layer.
- 35 5. The method of claim 4, wherein the catalyst comprises an organic peroxide.
- 40 6. The method of claim 5, wherein the organic peroxide comprises methyl ethyl ketone peroxide.
- 45 7. The method of claim 4, wherein the coating layer includes a graft initiator, wherein the graft initiator is operative to provide graft receptor sites on the insulating jacket layer.
- 50 8. The method of claim 7, wherein said graft initiator comprises a metallic salt.
9. The method of claim 8, wherein said metallic salt comprises silver perchlorate.
10. The method of claim 4, wherein said silane monomer comprises an amino-functional silane.

\* \* \* \* \*